

H. K. SANDELL.  
COMMUTATOR BRUSH.  
APPLICATION FILED MAR. 20, 1916.

1,222,999.

Patented Apr. 17, 1917.



Witnesses.

*John Tayler.  
Irvin G. Bowman.*

Inventor:

Henry K. Sandell,  
By Dymphna, Carlton Miles,  
At 1818.

# UNITED STATES PATENT OFFICE.

HENRY K. SANDELL, OF CHICAGO, ILLINOIS, ASSIGNOR TO HERBERT S. MILLS, OF CHICAGO, ILLINOIS.

## COMMUTATOR-BRUSH.

1,222,999.

Specification of Letters Patent. Patented Apr. 17, 1917.

Application filed March 20, 1916. Serial No. 85,322.

To all whom it may concern:

Be it known that I, HENRY K. SANDELL, a citizen of the United States, residing at 221 South Green street, Chicago, in the county 5 of Cook and State of Illinois, have invented a new and useful Improvement in Commutator-Brushes, of which the following is a specification.

My invention relates to certain new and 10 useful improvements in commutator brushes. The primary object of the invention is to provide a brush of high current-carrying capacity and long life and which will not wear the commutator. A further object of the 15 invention is to lighten the construction of the brush.

I find that the primary object of my invention is best obtained by a brush of cast metal. In the process of casting most metals 20 are brought to a more or less crystalline condition, and this crystalline structure seems to endow the brush with certain desirable properties as regards long life under sliding friction, and freedom from any tendency to 25 "seize" or unduly wear the surface of the commutator. While these attributes are to some extent common to all cast metal brushes they are, in the case of many metals, linked with disadvantageous properties such as 30 low conductivity, or a tendency to spark or to throw off incandescent particles.

I have found that by the use of certain metals or alloys I may obtain the desired 35 highly crystalline structure without sacrifice of any of the essential properties. The base metal which I have found best suited to these requirements is copper. For hardening the copper and giving to it the highest degree of crystalline structure without unduly lowering its conductivity I make use 40 of a certain proportion of antimony. I find it further desirable to use a proportion of a third metal or metals, such as nickel, lead and tin which appear to serve as a 45 "binder" or toughener, reducing the wear of the brush by preventing the disintegration of the contact surface under friction.

In applying these principles I obtain satis-

factory results from cast brushes of the following compositions:

| Parts by weight. |   |    |
|------------------|---|----|
| (1.) Copper      | 2 |    |
| Antimony         | 1 |    |
| (2.) Copper      | 8 | 50 |
| Antimony         | 2 | 55 |
| Tin              | 1 |    |
| (3.) Copper      | 4 |    |
| Antimony         | 2 |    |
| Lead             | 1 |    |
| (4.) Copper      | 8 | 60 |
| Antimony         | 4 |    |
| Nickel           | 2 |    |
| (5.) Copper      | 8 |    |
| Antimony         | 4 | 65 |
| Nickel           | 1 |    |
| Lead             | 1 |    |

All of these formulæ provide brushes of high conductivity and satisfactory wearing properties, both as regards the brush *per se* 70 and the commutator. For the service for which I have particularly designed my brushes, *i. e.*, for mechanically rectifying alternating current by a commutator driven from a synchronous motor, the last formula 75 seems to be the best. Formulae numbered 3 and 4 seem to be about equally good as between themselves, and both slightly inferior to formula 5, formula "two" is next best, and formula "one" least desirable, but 80 nevertheless quite serviceable.

In the particular service which I have mentioned it is not only desirable that the brush be of high conductivity in order that it may be of small cross-section and therefore of small depth without being necessarily of inordinate width, but it is further desirable that the weight of the brush be kept at the lowest point, for the reason that the most perfect commutator is not absolutely true, or at least does not remain so, and by its rotation at high speeds therefore tends to "kick" the brush outward as the points of eccentricity pass under the same. The time and angular travel of the commutator required to permit the brush to 85 90 95

again seat itself after having been kicked off will be a function of the mass of the brush and of the force exerted by the spring which feeds the brush inwardly. To increase the 5 tension of this spring is to increase the friction of and wear upon the brush and commutator, and it is therefore quite clear that the most advantageous results may be obtained by decreasing the mass of the brush. I accordingly prefer to construct my cast brush 10 in two sections; a wearing or surface section of highly conductive cast metal and a guide or supporting section of light metal such as aluminum, to which the conductor 15 wire or "pig-tail" is attached. These two sections are united, preferably by welding their abutting ends, so that the finished brush is an integral member, presenting the appearance shown by the accompanying drawing 20 in which proper legends are applied to the two sections and to the point at which they are joined.

In constructing such a brush the preferred mode of procedure is to first cast the aluminum guide section, the "pigtail" being cast 25 therein if desired, and to then lay this section in proper position in a brush mold, pouring in the molten alloy which is to constitute the operative portion of the brush. 30 The parts will thus be welded together in the act of casting and the brush may be removed from the mold and machined or ground to finished form as a unit.

What I claim as new and desire to secure 35 by Letters Patent is:

1. A brush cast from an alloy comprising copper, antimony and nickel.

2. A brush cast from an alloy comprising more than fifty per cent. of copper, about thirty per cent. of antimony, and more than 40 five per cent. of nickel.

3. A brush cast from an alloy comprising copper, antimony, nickel and lead.

4. A brush cast from an alloy comprising more than fifty per cent. of copper, and 45 about forty per cent. of antimony, nickel and lead taken together.

5. A brush cast from an alloy comprising about  $\frac{1}{2}$  copper, about  $\frac{1}{3}$  antimony, and about 50  $\frac{1}{6}$  of nickel and lead taken together.

6. A brush cast from an alloy consisting of 8 parts copper, 4 parts antimony and one part each of lead and nickel.

7. A brush comprising two abutting sections of different composition joined to 55 form an integral member, the wearing end section being of relatively heavy material and the guide end section being of relatively light material.

8. A metallic brush comprising two abutting sections of different metals joined to 60 form an integral member, the wearing end section being of relatively heavy metal and the guide end section of relatively light metal.

9. A metallic brush comprising two abutting sections of different metals joined to 65 form an integral member, the wearing end section being of copper alloy and the guide end section of aluminum.

10. An integral cast metal brush comprising a wearing end section of copper alloy and a guide end section of aluminum.

HENRY K. SANDELL.